

No. 691,297.

Patented Jan. 14, 1902.

J. L. SMITH & R. BEDFORD, JR.  
OPEN HEARTH STEEL PROCESS.

(Application filed Feb. 12, 1901.)

(No Model.)

2 Sheets—Sheet 1.



FIG. 1.

Witnesses:

*Fred W. Englehardt*  
*Percy C. Bowen.*

Inventors:

*John L. Smith,*  
*Robert Bedford, Jr.*  
*by Wilkinson & Fisher,*  
*Attorneys.*

No. 691,297.

Patented Jan. 14, 1902.

J. L. SMITH & R. BEDFORD, JR.

OPEN HEARTH STEEL PROCESS.

(Application filed Feb. 12, 1901.)

(No Model.)

2 Sheets—Sheet 2.



Witnesses:

Fried W. Englehardt  
Percy C. Bowen

Inventors:

John L. Smith,  
Robert Bedford, Jr.  
by Wilkinson & Fisher,  
Attorneys.

# UNITED STATES PATENT OFFICE.

JOHN LAW SMITH AND ROBERT BEDFORD, JR., OF EAGLESCLIFFE, ENGLAND,  
ASSIGNORS OF ONE-THIRD TO THE SOUTH DURHAM STEEL AND IRON  
COMPANY, LIMITED, OF STOCKTON-ON-TEES, ENGLAND.

## OPEN-HEARTH STEEL PROCESS.

SPECIFICATION forming part of Letters Patent No. 691,297, dated January 14, 1902.

Application filed February 12, 1901. Serial No. 47,067. (No specimens.)

*To all whom it may concern:*

Be it known that we, JOHN LAW SMITH and ROBERT BEDFORD, Jr., subjects of the King of Great Britain and Ireland, residing at Eaglescliffe, in the county of Durham, England, have invented certain new and useful Improvements in Open-Hearth Steel Processes; and we do hereby declare the following to be a full, clear, and exact description of the invention, such as will enable others skilled in the art to which it appertains to make and use the same.

This invention consists in a novel or improved process for producing steel in an ordinary type of open-hearth furnace adapted for the purpose by being provided with one or more dams so arranged that the hearth is divided into two or more compartments up to any required height and above which the said compartments merge into one large chamber which is common to all, whereby a charge of steel can be withdrawn from one or more compartments from time and time, while a bath of molten purified steel is left in one or more of the other compartments to remain on the furnace-bottom after tapping.

Before proceeding more particularly to describe the nature of our said invention we would first remark that it is a recognized advantage to retain on the bottom of an open-hearth furnace a bath or pool of steel left over from previous tappings, into which fresh charges of molten metal in an unpurified state—such as would be drawn from a blast-furnace, cupola, converter, or other suitable source of supply—can be poured from time to time without undue injury to the furnace-bottom; but the difficulty has been to effect this result in a practical manner, and the only methods hitherto devised which have been commercially used have been by tilting the furnace bodily or by other awkward means until a desired quantity of steel has run out. By such processes, if solid material is also to be used it must be charged into the bath of molten steel, which is cooled thereby and the process correspondingly retarded.

By our invention we not only charge the large compartment with unpurified molten metal, which is received into a bath of mol-

ten steel, but we also charge into the empty or practically empty compartment any desired quantity of solid materials—such as pig-iron, scrap metal, or other suitable material—where such charge is exposed to the heat of the furnace and raised to a suitable temperature before coming into contact with the molten steel which is pooled in the larger compartment, it being understood that by "unpurified" metal we refer to such metal as would run from a blast-furnace, cupola, or other source in a condition requiring further treatment for conversion into steel of the grade to be produced by the process in question.

Our process is a continuous one, and the steel is never drawn from the larger compartment until it is desired to shut down the furnace; but steel is from time to time drawn from the smaller compartment, this drawing off usually emptying the smaller compartment completely.

In the accompanying drawings, which represent an apparatus for carrying out our improved process, Figure 1 is a longitudinal section of an open-hearth furnace. Fig. 2 is a longitudinal section of the hearth, and Fig. 3 is a cross-section of the same.

Referring to Fig. 1, we propose to divide the hearth *a* into separate compartments by having an elevated portion *b* in the lining. This elevated portion *b* is made of similar material to the hearth itself, and this portion or partition-wall may be of any desired height, each compartment being furnished with its own tap-hole *c* at the bottom. In order to control the flow of the slag, which is liable to take place from the larger compartment into the smaller compartment as the latter is being emptied, we provide one or more channels *f* in the elevated portions *b*, transversely thereto. These channels may be of any desired width, depth, and shape. This construction allows the metal to flow from the larger compartment into the smaller compartment without disturbing the slag, which is allowed to settle in the manner required to protect and clear the steel. If the charge is large enough, one continuous bath will be formed, as shown by the line *x*. When the level of the steel is reduced to the line *y*,

two separate baths  $a'$  and  $a^2$  will be formed. By this construction the smaller bath may be completely emptied, leaving a bath of molten metal in the larger compartment up to the 5 line  $y$ .

The furnace is provided with the usual charging-doors  $d$  and the usual water-boshes or air-boxes  $e$  for cooling the hearth. If desired, an additional water-bosh or air-box 10 may be placed under the bank or wall  $b$  for cooling purposes.

While we have shown a furnace as divided into two compartments, it is obvious that we may use any number of these compartments 15 and that they may be of any desired size and shape.

In practice, the furnace being arranged and designed with two or more compartments, as described, but preferably with a larger and 20 smaller compartment only for convenience of description, it is intended that the following process should take place: The larger compartment being charged with a bath of molten steel left over from the previous tapping while the steel from the smaller compartment was run completely off, the process 25 consists in charging on the empty part of the furnace-hearth—*i. e.*, the aforesaid smaller compartment—after fettling, (if necessary,) 30 a quantity of ore or other oxids of iron—such as mill-scale, tap-cinder, and, if desirable, a certain quantity of limestone and scrap or other suitable materials, as circumstances and experience demands. This charging 35 of solid matter into the small empty compartment protects the hearth in this compartment from the overflow of molten metal from the large compartment, which overflow is not allowed to take place until the solid 40 material in the smaller compartment begins to melt. As soon as the scrap, ore, and the like has been brought up to a sweating heat 45 molten metal from the blast-furnace, converter, mixer, cupola, or the like is run into that compartment of the hearth containing

molten steel from the previous charge, and to which, if preferred, has been added oxid of iron, the whole mixing together and then flowing over the dam into the other compartment, coming in contact with the oxids of iron and scrap or the like, which are now at the best possible heat for making a chemical union. This submersion of the solid material in a molten bath causes a boil, after 55 which the charge in both compartments is worked in the usual way by fresh additions of iron ore and lime until the requisite purification and reduction of carbon has been effected.

When working scrap, less depth of bath is 60 required and less impurities are found. The slag covering the metal in a thinner sheet also permits the flame to act with greater intensity upon the metal.

The advantages are a continuous process 65 giving regular supplies to the mills at small intervals, a ready means of using the surplus scrap to advantage, increased output, and reduced wages and coal consumption.

Having thus described our invention, what 70 we claim, and desire to secure by Letters Patent of the United States, is—

The continuous process of manufacturing 75 steel, which consists in preparing a bath of molten steel in an open-hearth furnace provided with compartments, drawing off from time to time steel from one of said compartments, charging the empty compartment with solid materials, heating the furnace, allowing an additional charge of molten metal to run 80 into said furnace, making a bath which extends over all the compartments, and working the charge.

In testimony whereof we affix our signatures in presence of two witnesses.

JOHN LAW SMITH.

ROBERT BEDFORD, JUNIOR.

Witnesses:

GEORGE JAMES CLARKSON,  
EDWARD THOMAS ELEOAT.